

W. J. MERTEN.  
CORROSION RESISTING METAL ARTICLE AND METHOD OF MAKING SAME.  
APPLICATION FILED JAN. 4, 1918.

1,280,268.

Patented Oct. 1, 1918.

*Fig. 1.*



*Fig. 2.*



*Fig. 3.*



Inventor

William J. Merten

Witness

Chas. L. Griesbauer.

By Hull Smith Brock & West

Attorneys

# UNITED STATES PATENT OFFICE.

WILLIAM J. MERTEN, OF PITTSBURGH, PENNSYLVANIA, ASSIGNOR TO GEORGE D. BRECK, OF CLEVELAND, OHIO.

## CORROSION-RESISTING METAL ARTICLE AND METHOD OF MAKING SAME.

1,280,268.

Specification of Letters Patent.

Patented Oct. 1, 1918.

Application filed January 4, 1918. Serial No. 210,362.

*To all whom it may concern:*

Be it known that I, WILLIAM J. MERTEN, a citizen of the United States, residing at Pittsburgh, in the county of Allegheny and

5 State of Pennsylvania, have invented a certain new and useful Improvement in Corrosion-Resisting Metal Articles and Methods of Making Same, of which the following is a full, clear, and exact description, reference 10 being had to the accompanying drawings.

This invention relates to a method of treating certain articles of iron or steel whereby their resistance to corrosion or oxidation by the action of different adverse 15 agencies acting upon their respective surfaces may be augmented; and also relates to and includes certain articles and types of articles so treated and in which my invention is embodied.

20 Many expedients for inhibiting the rusting of iron have hitherto been suggested, but most of these have been restricted to articles which are normally used in a cold condition, as in the case of all machines and structural 25 materials, while very few expedients have been found for protecting iron or steel whose normal use is in the heated condition as is the case in stoves, furnaces, boilers, superheaters, economizers, pipes, valves, etc., especially in 30 cases where the two sides of the article are exposed to different oxidizing conditions, as, for example, the parts of a steam boiler where one side is in contact with heated water and the other with furnace gases.

35 The objects of my invention are: the provision of a new and improved method of treating devices of the character described for the purpose of enhancing their resistance to the corroding conditions to which they are

40 respectively subjected; the provision of a method of treating the respective surfaces of such devices as to obtain the maximum protective character of each and wherein the treatment of the one side shall have no inimical effect upon the condition or treatment of 45 the other side; the provision of such a combination of protective expedients that each shall be peculiarly suited to withstand the conditions to which it is exposed throughout the entire temperature range normally encountered in use; the provision of a protective method of such cheapness and convenience as to be susceptible of widespread use; the provision of certain articles and classes 55 of articles superior to any previously known

as regards their resistance to differing corrosive tendencies on their opposite sides; while further objects will appear as the description proceeds.

I have discovered that any treatment 60 which will be adequate at a given elevated temperature must be applied at a still more elevated temperature; and that if differing hot treatments are to be applied to different parts or sides of the article in question, those 65 treatments ought to be applied simultaneously in order to prevent the separate application of one treatment from either injuring the untreated portion of the article or damaging the treatment already applied; the 70 corollary of these propositions being that the two differing treatments should be such that both are most effectively performed at substantially the same elevated temperature.

As an example and not as a limitation of 75 my invention, I may treat the one surface of a pipe, tube, valve, sheet, box, plate, or receptacle by the process known as "sherardizing," simultaneously treating the opposite surface of the article in a mode to produce thereon a 80 coating of magnetic oxid. In the case of a tube, box, or receptacle which is to have moisture on the inside, as in a water tube boiler, steam chest, superheater, economizer, or the like, the sherardized surface will be 85 inside and the oxidized surface outside; in the case of the flues of a fire tube boiler the treatments would be reversed. And whatever particular treatments be employed the same are so situated that each will be 90 opposed to the deteriorating influence it can best withstand.

As a further description of a preferred embodiment of my invention, and assuming that I desire to treat a tube that is to be subjected to inside moisture and outside fire, I first remove all scale and other foreign matter from the tube, both inside and outside, place therein the necessary quantity of zinc dust, aluminum dust, copper filings or other 100 suitable metal or alloy, close the ends, and raise the whole to a low red heat, under oxidizing conditions, subsequently cooling slowly in a non-hydrating atmosphere. The desired production of magnetic oxid on the 105 exterior of the tube takes place at approximately the same temperature as does the adherent zinc-iron (or other alloy) coating on the interior, and both coatings will be permanent under all normal conditions of use 110

since always maintained at temperatures lower than that of their formation.

I do not assert inventorship of the above described process of sherardizing or that of 5 coating with magnetic oxid. I do not even restrict myself to those processes. What I 10 do declare to be my invention is the simultaneous performance on different parts of the same metal article of two hot processes 15 requiring the same approximate temperature, whereby the separate beneficial effects of those processes are secured as I have described; and it is wholly unimportant outside of these limits, what those processes are or whether they be new or old.

As another example, I may treat the one side of the article by a hot "galvanizing" process, or may coat the same by dipping in molten tin or zinc simultaneously with sherardizing, oxidizing or otherwise coating the 20 other side; or I may coat the interior and the exterior with different molten metals or fluxes.

The invention is also applicable to metals 25 other than iron, though of less importance in other connections.

In the drawings accompanying this application, which are to be read in an illustrative and not a limiting sense: Figure 1 is a 30 sectional diagrammatic view of part of a steam-generator embodying my invention; Fig. 2 is a view showing a step in my process; and Fig. 3 is a view of a different type of article embodying my invention.

In Fig. 1, 1 represents the tubes of a water tube boiler, 2 the header, 3 the steam reservoir, 4 the superheater, and 5 the steam pipe, all of which are sherardized interiorly 40 and coated with magnetic oxid exteriorly as described. 6 represents a steam valve whose interior is sherardized and whose exterior is not galvanized.

In Fig. 2, 10 represents the tube which is 45 being treated, and 11, 11, the caps by which the ends are closed and the two treatments kept apart.

Fig. 3 represents a culinary or other vessel made of iron and having for example, a cadmium-silver lining and a copper-zinc exterior coating, the two alloys having approximately the same melting points.

It will be understood that the foregoing description is illustrative rather than limiting and that many changes may be made

and numerous articles and treatments included within the scope of my invention.

Having thus described my invention what I claim is:—

1. The art of treating iron articles whose opposite sides are subjected to diverse corrod़ing influences which consists in subjecting those sides simultaneously to different corrosion inhibiting processes which require for their performance substantially the same elevated temperature. 65

2. The art of inhibiting corrosion in metal articles whose different parts are subjected to different corrod़ing influences, which consists in subjecting those parts simultaneously to two unlike hot processes, 70 each of which is adequate to inhibit the corrod़ing effect of the particular influence anticipated and both of which require approximately the same elevated temperature for their performance. 75

3. The art of inhibiting corrosion in iron articles whose opposite sides are subjected to heat and moisture respectively which consists in applying to the one side a hot surface treatment peculiarly resistant to moisture-corrosion and to the opposite side a hot surface treatment peculiarly resistant to heat corrosion, said treatments being of natures requiring substantially the same elevated temperature for their performance. 80

4. The art of inhibiting corrosion in iron articles whose opposite sides are subjected to heat and moisture, respectively, as in steam generating apparatus, which consists in applying comminuted zinc to that surface 90 which is to be subjected to moisture, heating the article so that its opposite side is exposed to oxidizing conditions to a temperature sufficient to melt the zinc, and finally cooling 95 the tube.

5. As an article of manufacture, a hollow metal article having upon its opposite sides a pair of dissimilar coatings whose application requires approximately the same elevated temperature. 100

6. As an article of manufacture a hollow iron article having one of its surfaces sherardized and its opposite surface covered with magnetic oxid.

In testimony whereof I hereunto affix my 105 signature.

WILLIAM J. MERTEN.